

A. L. STARK.  
METHOD OF MANUFACTURING ANTIMONY OXID.  
APPLICATION FILED DEC. 11, 1911.

1,096,468.

Patented May 12, 1914.



WITNESSES:

Oliver M. Kappeler.

Jes. F. Dhegin

INVENTOR -

Arthur L. Stark

BY J. B. Tay

# UNITED STATES PATENT OFFICE.

ARTHUR L. STARK, OF ELYRIA, OHIO, ASSIGNOR, BY MESNE ASSIGNMENTS, TO THE ENAMEL COMPANY OF AMERICA, OF ELYRIA, OHIO, A CORPORATION OF NEW YORK.

## METHOD OF MANUFACTURING ANTIMONY OXID.

1,096,468.

Specification of Letters Patent.

Patented May 12, 1914.

Application filed December 11, 1911. Serial No. 665,004.

To all whom it may concern:

Be it known that I, ARTHUR L. STARK, a citizen of the United States, and a resident of Elyria, county of Lorain, and State of Ohio, have invented a new and useful Improvement in Methods of Manufacturing Antimony Oxid, of which the following is a specification, the principle of the invention being herein explained and the best mode in 10 which I have contemplated applying that principle, so as to distinguish it from other inventions.

The object of the present invention is the provision of a method for the manufacture 15 of antimony oxid ( $Sb_2O_3$ ) from the sulfid in which form antimony chiefly occurs in nature, such sulfid being known in mineralogy as antimony glance or stibnite.

The present improved process is based 20 on the discovery that such antimony sulfid may be burned to the oxid and the sulfur simultaneously eliminated in the form of sulfur dioxide along with the other waste gases produced in such operation of burning.

25 Said invention then, consists of the steps hereinafter fully described and particularly pointed out in the claims.

The annexed drawing and the following description set forth in detail one approved 30 method of carrying out the invention, such disclosed mode, however, constituting but one of the various ways in which the principle of the invention may be used.

In said annexed drawings:—The single 35 figure there appearing, represents in more or less diagrammatic fashion, the apparatus adapted for carrying on my improved process.

Inasmuch as such apparatus is thus diagrammatically shown, its separate description is not deemed necessary, but such description may be incorporated in the explanation of the steps of the process proper, which will now be given.

40 The stibnite or antimony sulfid is preliminarily ground or pulverized, so as to be in the form of a fine powder. This disintegrated or powdered sulfid is then charged into a feeding hopper 1 provided with a screw 45 feed 2, by which it may be continuously fed into the air jet 3 of the blow pipe 4. Air is forced through such jet by a blower 5, while a pipe surrounding such jet, so as to form the outer tube of the blow pipe 4 is connected with a gas main 6. When the gas

thus supplied is ignited, the flame encircles the air jet 3 and the escaping air blast which carries the powdered sulfid. Such jet extends within one end of a furnace chamber 7, which preferably is not externally heated, the heat produced by the burning gas from the blow pipe ordinarily being sufficient to maintain a proper temperature within said chamber. It should also be noted that the antimony sulfid itself produces heat when burning, thus augmenting the heating effect of such burning gas. By thus decreasing the amount of fuel, in the form of gas, that is required for the burning operation just described, a considerable economy is effected over the prevailing method of oxidizing the metal to obtain the product under consideration. I have, furthermore, found that it is necessary to avoid too high a temperature in the furnace chamber, for the reason that the antimony oxid ( $Sb_2O_3$ ), which is formed as a result of the combustion of the sulfid in the manner described, passes through a liquid state before solidifying. If globules of this liquid are allowed to collect, they will, under the influence of a high temperature, oxidize still further, and, from the undesirable antimonic oxid. Accordingly, not only is the temperature in the furnace chamber properly regulated, but the walls of such chamber are spaced far enough apart to prevent the deposition of the antimony oxid thereon before it has passed through such liquid state and assumed the desired form of minute, solid particles. These latter, indeed, evince no great tendency to collect and remain in the furnace chamber, but are carried by the draft into the succeeding portions of the apparatus.

Directly following the furnace chamber is a series of cooling ducts 8 and associated settling chambers 9, through which such products are drawn, by means of a suction fan 10 and connecting pipes 11. The number of said ducts and settling chambers is immaterial, two being shown by way of illustration merely. Each chamber consists of a hopper-shaped box provided with a door through which the heavier antimony oxid may be removed after settling. The sulfur dioxide on the contrary, remains in the state of a gas throughout its progress through such chambers, and is thence discharged, along with the other waste gases from the combustion taking place in the retorts, by

the fan 10 into a dust collector, where the last trace of antimony oxid is removed. Such dust collector comprises a chamber 12 and another chamber 14 connected by cot-  
 5 ton tubes 13 or the like, the discharge pipe from fan 10 leading into said chamber 14, so that the products of combustion are finally passed into the latter before being dis- charged from the apparatus. These tubes 10 retain all solid particles, but permit the gaseous constituents to escape. Such solid particles, forming the remaining antimony oxid, are from time to time shaken from the tubes into the chamber 14 which serves as a  
 15 receptacle at the bottom of the dust collector from which such oxid may be removed as de- sired.

The blower 5 in connection with the suc-  
 20 tion fan 10 permits the gaseous products of combustion together with the oxidized antimony and sulfur to be passed in a constant and continuous stream of regulated velocity through the chamber 7 without permitting the adhesion of any of the particles of sulfid  
 25 or the oxid to the walls of said chamber, which is undesirable as previously ex- plained.

By reason of the regulation, which it is thus seen is rendered possible, I am enabled  
 30 to prevent the production of any but the desired antimony oxid ( $Sb_2O_3$ ), only an in- significant quantity of the higher oxid ( $Sb_2O_5$ ) being found in the resultant prod-  
 35 uct. In other words, by having the cham- ber arranged and constructed so as to im- mediately cool the oxid that are initially  
 40 formed upon ignition of the combustible mixture of air and gaseous hydro-carbon fuel and the sulfid suspended therein, only  
 45 the desired form of oxid is produced; and by having the walls of such chamber spaced sufficiently far apart to prevent the con- densation of such oxid thereon, the chang-  
 50 ing of the latter into the undesirable higher oxid is prevented. The operation, it will be seen, moreover, is a continuous one, and di- rectly converts the naturally occurring mineral into a commercial article without any  
 55 preliminary or intermediate treatment, save  
 60 for the grinding of the sulfid in order to permit it to be introduced into the blow pipe. It should further be noted that while the metal itself is poisonous in character and requires hence to be handled very care-  
 65 fully, the sulfid is free from this objection- able quality, and so may be utilized with impunity; while at the same time an actual economy in fuel results from the use of said sulfid owing to the fuel value of the sulfur  
 70 in the compound.

It will be understood, of course, that in practice the sulfur dioxid and other fumes, that form the waste products of the opera-  
 75 tion as described, will require to be con- ducted to a stack after escaping from the

dust collector. The tubes 13 of the latter will hence be desirably inclosed in a cham- ber (not shown) that is connected with a suitable stack.

Other modes of applying the principle of 70 my invention may be employed instead of the one explained, change being made as re- gards the process herein disclosed, provided the step or steps stated by any one of the following claims or the equivalent of such 75 stated step or steps be employed.

I therefore particularly point out and dis- tinctly claim as my invention:

1. The method of manufacturing anti-  
 80 mony oxid which consists in igniting pow- dered antimony sulfid while in a state of sus- pension, thereby producing a mixture of anti- mony oxid and sulfur dioxid; cooling such  
 85 oxid immediately after they are formed, so as to prevent the formation of antimonic  
 90 oxid; and then separating the antimony oxid from the other products of combustion.

2. The method of manufacturing anti-  
 90 mony oxid, which consists in igniting pow- dered antimony sulfid while in a state of sus- pension and out of contact with any sur- face, thereby producing a mixture of anti- mony oxid and sulfur dioxid; cooling such  
 95 oxid immediately after they are formed, so as to prevent the formation of antimonic  
 100 oxid; and then passing the products of combustion through a settling chamber and dust collector, whereby the antimony oxid is separated from the other products of combustion.

3. The method of manufacturing anti-  
 105 mony oxid, which consists in discharging a  
 110 combustible mixture of gases into a cham- ber, with powdered antimony sulfid sus- pended in such mixture; igniting such mix- ture of gases and sulfid thereby producing a  
 115 mixture of antimony oxid with sulfur di- oxid; cooling such oxid immediately after  
 120 they are formed, thus preventing the forma-  
 125 tion of antimonic oxid; and then separat- ing the antimony oxid from the other prod- ucts of combustion.

4. The method of manufacturing anti-  
 115 mony oxid, which consists in discharging a  
 120 combustible mixture of air and hydrocarbon  
 125 fuel into a chamber with powdered anti- mony sulfid suspended in such mixture; igniting such mixture and sulfid thereby pro-  
 130 ducing a mixture of antimony oxid and sul- fur dioxid; cooling such oxid immediately after they are formed, thus preventing the forma-  
 135 tion of antimonic oxid; and then separat- ing the antimony oxid from the other prod- ucts of combustion.

5. The method of manufacturing anti-  
 130 mony oxid, which consists in discharging a  
 135 combustible mixture of air and gaseous hy- drocarbon fuel into a chamber, with pow- dered antimony sulfid suspended in such

mixture; igniting such mixture and sulfid, thereby producing a mixture of antimony oxide and sulfur dioxid; cooling such oxids immediately after they are formed, thus preventing the formation of antimonic oxide; and then passing the products of combustion through a settling chamber and dust collector, whereby the antimony oxide is separated from the other products of combustion.

6. The method of manufacturing antimony oxide, which consists in discharging a combustible mixture of air and gaseous hydrocarbon fuel into a chamber with powdered antimony sulfid suspended in such

mixture; igniting such mixture and sulfid, thereby producing a mixture of antimony oxide and sulfur dioxid; cooling such oxids immediately; and then passing such products of combustion through a settling chamber and dust collector, whereby the antimony oxide is separated from the other products of combustion. 20

Signed by me this 6 day of December, 1911.

ARTHUR L. STARK.

Attested by—

L. S. FAUVER,  
L. B. FAUVER.